

No. 664,024.

Patented Dec. 18, 1900.

P. J. MORAN.

STREET PAVING.

(Application filed Apr. 3, 1900.)

(No Model.)



Quartz or hard stone  
Limestone  
Portland cement



Witnesses  
C.W. Heiskell  
T.F. Kelley

Inventor  
Patrick J. Moran  
by J.H. Weatherford  
his atty.

# UNITED STATES PATENT OFFICE.

PATRICK J. MORAN, OF MEMPHIS, TENNESSEE.

## STREET-PAVING.

SPECIFICATION forming part of Letters Patent No. 664,024, dated December 18, 1900.

Application filed April 3, 1900. Serial No. 11,376. (No model.)

*To all whom it may concern:*

Be it known that I, PATRICK J. MORAN, a citizen of the United States, residing at Memphis, Shelby county, State of Tennessee, have 5 invented certain new and useful Improvements in Street-Paving, of which the following is a specification.

My invention relates in general to street-paving, and more especially to that class 10 known as "concrete" paving, in which a bonding material—such as cement, asphalt, or the like—is used to bond together the paving material proper.

Briefly resuming, in the attempt to provide 15 a good paving material many different materials and combinations of materials have been tried with varying success. Among the first of these are natural gravels having a clay binding material, which are now largely in 20 use, but which because of the poor character of the binding materials will not stand excess of wet or dry weather, and therefore are not entirely satisfactory. Macadam for the same reason is not a thorough success, and the 25 minds of men have naturally turned to other fields which follow more or less closely the lines set out by these materials. In the manufacture of composite pavements it has hitherto been customary to use broken or granulated rock and to bond them together with 30 Portland cement or the like and to finish off the surface with a combination of sand and cement to give a smooth surface. This mass, being of unequal composition, cracks and 35 breaks and is otherwise very unsatisfactory in that it gives a surface that is originally smooth and that under wear becomes more so. Later attempts to improve these have resulted in the use of finely crushed or pulverized 40 stone as a wearing-surface and in the use of gritty substances as a top-dressing. These while of value for sidewalks have no value whatsoever as street-paving proper in that they all present a surface that is excessively 45 smooth to horses and gives them no secure foothold whatsoever.

The objects of my invention are to provide 50 a durable wearing-surface for street-paving which will at one and the same time be smooth for the wheel-tread and yet afford sufficient

foothold for horses, one which may be laid with a correct wearing-surface and if not so laid will assume and preserve same under continuous wear, and one which will give the maximum of use with the minimum of attention and when necessarily disturbed may be repaired with minimum trouble and expense. I accomplish these objects by making the pavement of a comparatively hard material of sensible size interspersed with a relatively 55 soft material and a binder, or with the relatively soft binder alone, the hard material being of sufficient size to leave, when used with the binder alone, small spaces filled with the binder, which having small resistance to wear 60 wears down slightly and gives a surface which is of the nature of good macadam or gravel and presents a foothold for the horse and as well a smooth surface for the carriage-wheel of large diameter. Where an additional material is used with the binder, it gives slightly- 65 larger spaces and a slightly-rougher surface, as will be more fully set out in the general description. I further accomplish these objects by reinforcing the pavement at the 70 points of maximum wear.

Referring now to the drawings, in which like letters of reference indicate like parts in all the views, Figure 1 is a sectional perspective of a portion of a city street, showing 80 sidewalks, curbs, and the street proper embodying the principal features of my invention. Fig. 2 is a section of the paving on an enlarged scale. Fig. 3 is a like section showing a modification in composition. Fig. 4 is 85 a vertical section showing Fig. 3 under wear.

In the drawings, A is a section of street, showing my paving. B is a street-car rail; C, the street-curb, and D the sidewalk.

Since the greatest wear in any street comes 90 near the center of same, I reinforce same or make it heavier at that point. If the street is unbroken by car-tracks, I make this gradual from the center to the sides. If, however, the street be one, as shown, with street-car 95 rails, I find that the wear is greatest within two to three feet on the outside of the car-track and that from that point out decreases rapidly for a short distance and then decreases in a much slower ratio to the 100

street-curb. To increase the life of the paving, I therefore reinforce it uniformly from the rail B to a point E about two feet distant therefrom and then make a rapid drop, as shown, to the top level proper, sloping it thence gradually to the curb.

Taking up now the construction of the pavement, or rather of the wearing-surface for the pavement, I use a hard stone—such as granite, flint, quartz-rock, iron slag, or hard river-gravel washed clean, broken to pass through a two to two-and-one-half inch ring—mixed with a softer stone, such as Georgia bastard limestone, broken to about the same size or preferably slightly smaller, with sufficient sand to fill the voids and all bonded together with a good grade of cement, which is preferably Portland. I find that the proportion used in ordinary concrete—viz., six of stone, two of sand, and one of cement—is about the best mixture, and of the stone one-half to two-thirds is to be the hard granite and the remainder the softer stone.

In Fig. 3 I have shown a section of pavement as first laid, in which K represents the soft-stone constituent and L the hard or granite. In Fig. 4 I show the same pavement after hard usage, showing that the granite L has worn comparatively little, while the limestone K has worn sufficiently to give slight depressions G between the adjacent high points H. The object of combining these stones of different hardness is to provide these slight depressions and to prevent the pavement wearing slick under continuous wear. These depressions G are prevented from becoming excessively deep by the hardness of the adjacent points H of the granite L. I find, too, that where the crushed granite is sufficiently large (about two and one-half inches) it is possible to secure the same effect, though not in so satisfactory a degree, by binding the granite alone and sufficient sand to fill the voids with a good cement binder or, in other words, to make the top-dressing for the street of coarse-stone concrete instead of finishing it with a smooth fine-crushed stone and sand-facing, as is now commonly done. In this case the depressions G, as shown in Fig. 2, are in the cement and sand part of the concrete, the high points H being the tops of the granite cubes.

While I have in this description confined myself to the surface of the pavement only, I prefer to make the pavement homogeneous, as shown—in other words, to use the same size stone I at the top as those J at the bottom, though this is not necessarily an essential feature of my invention. In either case this pavement possesses the essential features of correct wearing-surface, great strength, imperviousness to water, and is easy to repair.

The correct wearing-surface, which is the first essential, is obtained, as before stated, by the uneven wear of the materials of construction, which uneven wear gives slight de-

pressions between the hard points of the hardest material and permits foothold for the horses' feet. The wear is kept even by the fact that after a certain amount of depression has been reached the wheels grind only the projecting material and with the aid of the wear from the horses' feet wear this as rapidly as the horses' feet are able to do the softer material. This surface is practically as smooth to the large-diameter wheel as the best brick, asphalt, or other known pavement, with the additional advantage of absolute hardness to prevent the sinking of the wheel under heavy loads, as in asphalt, by its wavy displacement or on brick by the bodily displacement of same and at the same time giving foothold for the horse, thus permitting great increase in the amount of load which can be hauled over it by any given team. The great strength is given by the uniform nature of the material providing equal expansion, but more especially by the thorough and strong bonding of the large pieces of stone with the cement and sand, the large pieces giving a thorough and interlocking bond between the parts and the feature of imperviousness to water protecting it practically from all exposure to action by the atmosphere.

Imperviousness to water is an important factor in that not only is the paving itself protected from action by the water, but the foundation underneath is protected both from addition to its moisture or loss of what it contains by evaporation, a firm foundation for the pavement being thus preserved at all times. It is absolutely sanitary in that nothing offensive can permeate it to remain and throw out its noxious odors, and by reason of its hardness it can be swept perfectly clean and all such material removed. Its wear is so immaterial that no dust from it is added to the street-sweepings, and as no loose sand is necessary on its surface this trouble is also escaped. The last feature (ease of repair) is by no means the least important in street-paving, which is subject to continual tearing up and replacing in the laying of water-pipes, sewers, &c. In my pavement it is only necessary to recrush the concrete and mix with cement and sand to bond it together, then to tamp it in place even with the surface of the street, and the work is done, the replaced portion being practically as good as when first laid and being equally as impervious to water, and by reason of its strength and perfect bond with the original pavement is in no danger of sinking under heavy loads.

In the claim I have used the word "stone" generically, as including all classes of material—such as crushed stone, crushed granite, iron slag, gravel, &c.—as distinguished from a narrow specific class.

What I claim, and desire to secure by Letters Patent of the United States, is—

As a surface-layer for street-paving, a con-

crete comprising the combination with a coarse hard stone and a coarse softer stone, both broken approximately to pass through a two-and-one-half-inch ring, of a binding

5 material of sand and cement, mixed in the proportions of about three parts each of the stone, two of sand, and one of cement.

Gross, 220, 244, Oct. 7, 1879, Paving, Concrete.

In testimony whereof I have signed my name to this specification in the presence of two subscribing witnesses.

PATRICK J. MORAN.

Witnesses:

C. W. HEISKELL,

T. F. KELLEY.

Murphy, 219, 501, Sept. 9, 1879, "

Amberg, 291, 482, Jan. 8, 1894, "

Pain, 539, 821, May 28, 1895, Stone Pavements

Lee, 188, 645, Mar. 20, 1877, Concrete Pavements

Mills, 238, 419, Mar. 1, 1881,

Richardson, 161, 550, Mar. 30, 1875, Paving, Concrete,

Abbott, 139, 848, June 17, 1873, "

Reissue patent to Dean, 6570, Aug. 3, 1875, "

McKinley, 278, 031, May 22, 1883, "